

## UNITED STATES PATENT OFFICE

2,203,641

## STABLE EMULSION

Roland Kapp, Newark, N. J., assignor to National  
Oil Products Company, Harrison, N. J., a cor-  
poration of New Jersey

No Drawing. Application October 23, 1937,  
Serial No. 170,595

16 Claims. (Cl. 252—6)

The invention relates, in general, to emulsified metallic soaps and, in particular, to emulsions of water-insoluble salts of naphthenic acids or naphthenic acid esters.

5 The water-insoluble soaps, and more particularly the water-insoluble naphthenates of the polyvalent metals and derivatives thereof, have been found to possess valuable properties and characteristics which adapt them to many practical and potential uses in the industrial arts. These salts are admirably suited for preserving fibrous materials, such as wood, paper, textiles, etc., against rot and decay and for waterproofing and weatherproofing the above-named fibrous as 10 well as porous materials such as concrete, stone, etc. These salts have also found extensive use in the manufacture of cutting oils, sprays, insecticides, fungicides, germicides, and the like. In the preparation of solutions or compositions 15 containing the polyvalent metal salts of naphthenic acids or derivatives thereof, it has been necessary to employ organic solvents in dissolving, swelling or dispersing these salts in view of their extreme resistance to wetting by water and 20 water-soluble wetting and emulsifying agents. This factor has restricted the use of these salts as in many instances the presence of organic solvents is prohibited or highly undesirable. Moreover, organic solvents are expensive and 25 greatly increase the cost of manufacturing compositions of the type referred to above.

The general object of the invention is to obviate the foregoing and other disadvantages.

A specific object of the invention is to provide 30 a fluid, organic solvent-free composition containing a polyvalent metal salt of naphthenic acids.

Another object of the invention is to dispense with the use of organic solvents in the preparation 35 of compositions containing polyvalent metal salts of naphthenic acids.

Other objects of the invention will in part be obvious and will in part appear hereinafter.

It has now been discovered that polyvalent metal salt of naphthenic acids or naphthenic 40 acid esters may be emulsified to form stable oil-in-water type emulsions. According to the invention such emulsions are produced by employing as the emulsifier a sulfation product of an ester of naphthenic acids with an unsaturated 45 compound containing 8 or more carbon atoms selected from the group consisting of monohydric fatty alcohols, hydroxy fatty acids and hydroxy fatty esters.

The invention accordingly comprises the several 50 steps and relation of one or more of such steps

with respect to each of the others, and a composition of matter possessing the characteristics, properties and relation of components, all of which will be exemplified in the following detailed disclosure, and the scope of the invention 5 will be indicated in the claims.

The expression "naphthenic acids" is employed herein to connote the mixture of acids of that name currently obtained in petroleum refining, as well as the naphthenic acid or acids which are 10 synthetically prepared or otherwise obtained. It is preferred, however, to use the naphthenic acids derived from the refining of petroleum in view of their relatively low cost.

The metallic salts which can be emulsified according to the invention comprise the naphthenates of polyvalent metals, such for example, as naphthenates of lead, copper, aluminum, tin, zinc, mercury, etc., or derivatives of these soaps, such as the lead, copper, aluminum, etc. salts 20 of an ester of naphthenic acids with ricinoleic acid or castor oil, or any combination of two or more of these or other salts. For the purpose of this invention the expression "salt of a naphthenic compound" will be used to generically 25 include the straight naphthenic acid salts as well as the salts of naphthenic acid esters of the aforementioned type. The lead and copper naphthenates or lead and copper salts of naphthenic acid esters, as well as a combination of these two 30 salts, are particularly well suited for emulsification according to the present invention. The metallic naphthenates or derivatives thereof to be emulsified according to the invention may be produced by the reaction of naphthenic acids or 35 esters on suitable salts of various metals, or by any other suitable method known to the art.

The production of stable emulsions of the above referred to naphthenates may be achieved, according to the invention, through the use of 40 new and specially prepared emulsifiers which comprise the sulfated esters of naphthenic acids with an unsaturated compound, containing 8 or more carbon atoms, selected from the group consisting of fatty alcohols, such as oleyl alcohol, 45 hydroxy fatty acids, such as ricinoleic acid, and hydroxy fatty esters, such as castor oil. In practice the sulfated esters of naphthenic acids with castor oil or ricinoleic acid have proven to be of particular value and their use in instant case is 50 highly preferred. The new emulsifiers per se, which are employed in carrying out the present invention, are fully disclosed and claimed in my co-pending application for U. S. Letters Patent, Serial Number 170,596, filed October 23, 1937. 55

For a fuller understanding of the nature and objects of the invention, reference should be had to the following examples which are given merely to illustrate some of the compositions of the invention and the method of making the same, and in no way should they be construed in a limiting sense.

*Example I*

10 One part of lead naphthenate, prepared by known methods, is mixed with two parts of an emulsifier consisting of the sulfated ester of naphthenic acid and castor oil.

15 When one part of this mixture is stirred into 9 parts of water, a stable emulsion is formed. The lead emulsion thus produced can be used in emulsifying cutting oils, in metal stamping or drawing lubricants or in other industrial applications.

*Example II*

20 One part of copper naphthenate is mixed with one part of the sulfated ester of naphthenic acids with castor oil.

25 A 2 to 5% emulsion of the above mixture is useful as a fungicide, wood preservative, etc.

*Example III*

30 One part lead naphthenate and two parts copper naphthenate are mixed with six parts of the sulfated ester of naphthenic acids with castor oil.

35 A 1-10% emulsion of the above mixture is useful as a fungicide, wood preservative, etc.

*Example IV*

35 One part of a lead salt of an ester of naphthenic acids with ricinoleic acid is mixed with two parts of the sulfation product of an ester of naphthenic acids with ricinoleic acid. This mixture is then stirred into the desired quantity of water.

*Example V*

40 A mixture of one part aluminum naphthenate and three parts sulfated oleyl naphthenate is emulsified into water to produce a 10% emulsion. This emulsion is useful in textile treatments and 45 for water-proofing of various fibrous and mineral materials.

*Example VI*

50 The oleyl naphthenate of Example V is replaced by the sulfated ester of naphthenic acids with ricinoleic acid.

55 The proportions of metallic naphthenates and their derivatives and emulsifiers given in the above examples are merely illustrative, and it must be understood that emulsions satisfactory for various purposes can be produced with the use of a greatly reduced percentage of emulsifier in the finished mixture. Such emulsions may not remain stable as long as emulsions containing a higher percentage of emulsifier, but it is not always desirable to have a perfectly stable emulsion, as for example, in the field of insecticides, the use of emulsions having reduced or temporary stability is desirable. For such applications, the percentage of emulsifier in the mixture can therefore be greatly reduced. While for all practical intents and purposes the objects of the invention may be fully realized by the use of the hereinbefore disclosed emulsifiers, whether containing moisture or not, it has been found that the stability of the emulsions of the invention may be enhanced if the anhydrous form of the emulsifier is employed.

70 The percentage of water in the emulsion can 75 also be varied within wide limits, according to

the type and viscosity of emulsion which seems desirable for the particular use contemplated. Such emulsions, for example, may contain as little as 50% water or less, while others may be made with as much water as is deemed necessary 5 or desirable. Since the insoluble metallic naphthenate emulsions or emulsion of their derivatives produced according to this invention are of the oil-in-water type, it is evident that their dilution with water offers no difficulty.

10 Since certain changes in carrying out the above process and certain modifications in the composition which embody the invention may be made without departing from its scope, it is intended that all matter contained in the above description 15 shall be interpreted as illustrative and not in a limiting sense.

It is also to be understood that the following claims are intended to cover all of the generic and specific features of the invention herein described 20 and all statements of the scope of the invention which, as a matter of language, might be said to fall therebetween; and that they are intended to be inclusive in scope and not exclusive, in that if desired other materials may be added to my 25 novel composition of matter herein claimed without departing from the spirit of the invention. Particularly it is to be understood, that in said claims ingredients or components recited in the singular are intended to include compatible mixtures of said ingredients wherever the sense permits.

Having described my invention, what I claim as new and desire to secure by Letters Patent is:

1. A stable emulsion comprising a polyvalent 35 metal salt of a naphthenic compound, water and a sulfation product of an ester of naphthenic acids with an unsaturated compound, containing 8 or more carbon atoms, selected from the group consisting of monohydric fatty alcohols, hydroxy 40 fatty acids and hydroxy fatty esters.

2. A stable emulsion comprising a lead naphthenate, water and a sulfation product of an ester of naphthenic acids with an unsaturated compound, containing 8 or more carbon atoms, selected from the group consisting of monohydric fatty alcohols, hydroxy fatty acids and hydroxy 45 fatty esters.

3. A stable emulsion comprising a copper naphthenate, water and a sulfation product of an ester 50 of naphthenic acids with an unsaturated compound, containing 8 or more carbon atoms, selected from the group consisting of monohydric fatty alcohols, hydroxy fatty acids and hydroxy fatty esters.

4. A stable emulsion comprising a lead naphthenate, copper naphthenate, water and a sulfation product of an ester of naphthenic acids with an unsaturated compound, containing 8 or more carbon atoms, selected from the group consisting 60 of monohydric fatty alcohols, hydroxy fatty acids and hydroxy fatty esters.

5. A stable emulsion comprising a polyvalent metal salt of a naphthenic compound, water and a sulfation product of an ester of naphthenic 65 acids with oleyl alcohols.

6. A stable emulsion comprising a polyvalent metal salt of a naphthenic compound, water and a sulfation product of an ester of naphthenic acids with ricinoleic acid.

7. A stable emulsion comprising a polyvalent metal salt of a naphthenic compound, water and a sulfation product of an ester of naphthenic acids with castor oil.

8. A stable emulsion comprising lead naph-

thenate, water and a sulfation product of an ester of naphthenic acids with castor oil.

9. A stable emulsion comprising copper naphthenate, water and a sulfation product of an ester of naphthenic acids with castor oil.

10. A stable emulsion comprising aluminum naphthenate, water and a sulfation product of an ester of naphthenic acids with ethyl alcohol.

11. A process of producing stable emulsions which comprises mixing a polyvalent metal salt of a naphthenic compound with a sulfated ester of naphthenic acids with an unsaturated compound selected from the group consisting of monohydric fatty alcohols, hydroxy fatty acids and hydroxy fatty esters and stirring the mixture into an aqueous vehicle.

12. A process according to claim 11, wherein an anhydrous sulfated ester is employed.

13. A water-dispersible composition comprising a polyvalent metal salt of a naphthenic compound and a sulfation product of an ester of naphthenic acids with an unsaturated compound containing 8 or more carbon atoms selected from the group consisting of monohydric fatty alco-

hols, hydroxy fatty acids and hydroxy fatty esters.

14. A water-dispersible composition comprising lead naphthenate and a sulfation product of an ester of naphthenic acids with an unsaturated compound containing 8 or more carbon atoms selected from the group consisting of monohydric fatty alcohols, hydroxy fatty acids and hydroxy fatty esters.

15. A water-dispersible composition comprising copper naphthenate and a sulfation product of an ester of naphthenic acids with an unsaturated compound containing 8 or more carbon atoms selected from the group consisting of monohydric fatty alcohols, hydroxy fatty acids and hydroxy fatty esters.

16. A water-dispersible composition comprising lead naphthenate, copper naphthenate and a sulfation product of an ester of naphthenic acids with an unsaturated compound containing 8 or more carbon atoms selected from the group consisting of monohydric fatty alcohols, hydroxy fatty acids and hydroxy fatty esters.

ROLAND KAPP.